

## UNITED STATES PATENT OFFICE

2,151,300

## MINERAL OIL COMPOSITION

Robert C. Moran, Wenonah, and Alfred P. Koza-cik, Woodbury, N. J., assignors to Socony-Vacuum Oil Company, Incorporated, New York, N. Y., a corporation of New York

No Drawing. Application December 16, 1938,  
Serial No. 246,244

29 Claims. (Cl. 87—9)

This invention has to do in a general way with mineral oil compositions and is more particularly related to mineral oil compositions of the lubricant type to which an agent has been 5 added for the purpose of improving the oil in certain respects. The present application is a continuation in part of our copending application Serial No. 158,738, filed August 12, 1937.

It is the object of this invention to provide a 10 novel class of improving agents for use in mineral oil fractions of the class described and further to provide improved mineral oil compositions containing such improving agents.

As is well known to those familiar with the 15 art, modern practice in the manufacture of lubricants requires the addition of various agents to the mineral oil base stocks for the purpose of adding new properties, improving inherent properties, or inhibiting the development of undesirable properties latently present within the oil. It is customary, for example, where the lubricant is to be subjected to extremely high bearing pressures, such as are encountered in hypoid gears, to add an agent which will increase the 20 load-carrying capacity of the oil. Such agents are known as extreme pressure or E. P. agents. It is also customary where the oil is to be used under oxidizing conditions as in an automobile crank case to add an agent which will inhibit 25 the deleterious effects of oxidation on the oil. In this latter regard it has been found that motor oil compositions, particularly those prepared from crude oil fractions of high paraffinicity or from oils which have been solvent-refined, when 30 used in engines employing bearing surfaces of cadmium-silver, copper-lead, high-lead babbitts and similar alloys are prone to cause corrosion of such bearings. This apparently arises from the formation of acidic reaction or oxidation 35 products under the conditions of use. Additive agents which when added to the oil prevent such corrosive action fall into the general class of materials known as oxidation inhibitors or anti-oxidants and may be more specifically classified 40 as corrosion inhibitors.

Among the more successful compounds which have been developed for use as corrosion inhibitors are the esters of phosphorous acid, which we may also term organic phosphites. Besides 45 functioning as corrosion inhibitors or anti-oxidants in mineral oil fractions refined for motor lubricants and the like, these compounds also find use as extreme pressure agents in lubricants for hypoid gears, etc.

50 Although the esters of phosphorous acid, as

indicated above, have proved to be highly effective in improving certain properties of mineral lubricating oils, they have one disadvantage in that an oil containing an ester of phosphorous acid or an organic phosphite tends to stain metal 5 containers, particularly tin-coated metal containers, when stored therein at atmospheric temperature. With increase in temperatures this staining becomes accelerated. Thus an S. A. E. 10 20 motor oil containing 0.25 per cent of tri-tertiary amyl phenyl phosphite will cause a visible stain in a tin-coated container in about twenty-one days when stored at 120° F. and in about three days when stored at 160° F.

The effect of customer reaction when discovering such staining is obvious, particularly when much motor oil is sold in containers intended for re-use by the customer for other purposes. Of more actual importance is the fact that the staining is accompanied by a darkening of the oil, 15 which is also highly objectionable from a marketing standpoint. Furthermore, the unit of effectiveness of the oil with respect to the purpose for which the ester of phosphorous acid is 20 added is decidedly impaired, since the staining 25 of the tin-coated container and the darkening of the oil are the results of deterioration of the ester of phosphorous acid.

Since all known esters of phosphorous acid or 30 organic phosphites are inherently unstable, particularly in the presence of moisture and more particularly in the presence of acids or alkalies, it is obvious that the serious objections to such esters or phosphites for improving certain characteristics of mineral oils, particularly motor oils, 35 cannot be overcome without improving the inherent stability of the esters. This invention is specifically directed to the solution of this problem and is predicated upon the discovery that the stability of esters of phosphorous acid, particularly when used in small concentrations as 40 improving agents for mineral oils, can be decidedly increased by means of a relatively small proportion of an oil-soluble organic amine.

Our invention, therefore, contemplates as an 45 improving agent for mineral oils a composition comprising an organic phosphite or ester of phosphorous acid and an oil-soluble organic amine in sufficient amount to stabilize the ester or phosphite against deterioration or hydrolysis when 50 added to the oil. It will be seen that with such a composition the ester is protected against deterioration both prior to and after its addition to the oil. It will be understood, however, that the organic phosphite and the amine may be 55

added to the oil separately, and our invention therefore contemplates a mineral oil composition containing an ester of phosphorous acid in sufficient amount to stabilize the oil against the deleterious effects of oxidation (such as corrosion of alloy bearings, etc.) or in sufficient amount to impart extreme pressure characteristics to the oil and an oil-soluble organic amine in sufficient amount to bring about substantial stability and retard staining action of the phosphorous acid ester upon tin-coated containers.

Broadly, therefore, it will be seen that our invention comprehends two essential constituents, namely, an organic phosphite and an oil-soluble organic amine, which may be blended together in suitable proportions and added to the oil as a compounded oil-improving agent or which may be independently added to the oil in the required proportions to give in both events an improved mineral oil composition.

The organic phosphites or esters of phosphorous acid contemplated by this invention may be represented as a class by the general formula:



in which R' represents an aryl or an alkyl radical; R represents hydrogen, aryl, or alkyl radicals; and X represents oxygen or sulfur. The term "aryl" as employed herein is inclusive of unsubstituted aromatic hydrocarbon radicals and aromatic hydrocarbon radicals in which one or more nuclear hydrogen atoms have been substituted with an aliphatic hydrocarbon group, for example,

Within the general class of organic phosphites discussed above, preference is given to the triesters of phosphorous acid, both aryl and alkyl. Illustrative of the triaryl phosphites may be mentioned triphenyl phosphite, tri-tertiary amyl phenyl phosphite, tri-tertiary butyl phenyl phosphite, tricresyl phosphite, tribeta naphthyl phosphite, etc. Illustrative of trialkyl phosphites are tributyl phosphite, tri-isomethyl phosphite, etc. Although preference is given to triesters of phosphorous acid of the type represented by the foregoing examples, it is again emphasized that our invention is not restricted thereto but encompasses phosphites (including thiophosphites) as a general class.

As to the amine constituent of the oil-improving agent and improved mineral oil composition contemplated herein, preference is given to the cyclohexylamines (di- and mono-), dicyclohexylamine being particularly preferred. The invention, however, is not restricted to any particular amine but is inclusive of oil-soluble amines in general. Representative examples of amines which have proved to be highly effective are lecithin, morpholine, orthotoluidine, triethanolamine, triethanolamine stearate, paraphenylene diamine, paratoluidine, beta naphthylamine, di-anisidine, orthotolidine, para,para-diamino diphenylmethane, phenyl hydrazine, amyl amine, aniline, diamylamine, and hexamethylenetetra-amine. Other amines of somewhat less effectiveness are tetramethyl thiuram disulfide, para-phenetidine, ethyl alphanaphthylamine, ortho-amino-diphenyl, ortho-amino-phenol, methyl anthranilic acid, dibeta naphthylamine, and para-nitraniline.

The range of proportions of the organic phos-

phite and the amine which may be employed in compounding the mineral oil-improving agents or which may be added to a mineral oil independently to provide the improved mineral oil compositions contemplated herein may be varied over relatively wide limits. We may employ, for example, equal parts of the phosphite and the amine, or the amount by weight of amine used may be as little as 0.25 per cent of that of the phosphite. Where the phosphite is to be used for the purpose of inhibiting corrosion in a motor lubricant it appears that an amount of amine in excess of about 50 per cent the weight of the phosphite is likely to affect the corrosion-inhibiting power of the phosphite, and for such use it is therefore preferable to use the amine in amounts not exceeding 50 per cent the weight of the phosphite used. For general purposes the quantity of amine may be varied from about 0.4 per cent to about 20 per cent the weight of the phosphite (or from about 0.001 per cent to about .05 per cent the weight of the oil), with proportions of from about 0.4 per cent to about four per cent (from about .001 per cent to about .01 per cent based on the oil) considered as preferred. Very satisfactory corrosion inhibiting compositions are obtained with phosphite of the type disclosed herein, such as tritertiary amyl phenyl phosphite or tritertiary butyl phenyl phosphite, for example, containing from about 2 per cent to about 3 per cent of a cyclohexylamine, preferably the dicyclohexylamine. It will be understood, of course, that the solubility of a particular amine in mineral oil is a factor which must be considered in determining the quantity of that amine used in the oil and, consequently, also affects the quantity which will be employed in a phosphite and amine composition for use in the oil.

The quantity of the composite organic phosphite and amine inhibiting agent added to the oil or the combined percentage of phosphite and amine independently added to the oil may also be varied over relatively wide limits, depending upon the oil, the proportions of phosphite and amine used, and the purpose for which the improving agent is added. In general it appears that satisfactory results will be obtained in inhibiting the corrosive action of motor lubricants with the use of a combined amount of phosphite and amine equal to from about 0.1 per cent to about 5 per cent the weight of the oil.

An interesting observation which we have made regarding the combined use of an organic phosphite and an amine is that the improved results obtained are apparently not due to any antioxidant effect of the amines added, since many of the most effective amines, particularly cyclohexylamine, are not effective antioxidants according to tests commonly used for determining antioxidant ability of additive compounds in oil.

The following examples constitute specific illustrations of the invention contemplated herein and will serve to amplify the generalizations made hereinabove.

#### EXAMPLE 1

As already mentioned, an S. A. E. 20 oil containing 0.25 per cent of tri-tertiary amyl phenyl phosphite or 0.25 per cent of triphenyl phosphite, when stored at 120° F., produces a visible stain when in contact with the tin coating of the container in about twenty-one days. Samples of the same oil were then blended with 0.25

per cent of these same phosphites and 0.05 per cent or less (based on the oil) of various amines and subjected to the same test, and in no case was any staining discernible at the end of 104 days of storage when the test was discontinued. The following representative amines were used in this series of tests: (1) cyclohexylamine, (2) di-cyclohexylamine, (3) lecithin, (4) morpholine, (5) orthotoluidine, (6) triethanolamine, (7) triethanolamine stearate, (8) paraphenylenediamine, (9) paratoluidine, (10) beta naphthylamine, (11) dianisidine, (12) orthotolidine, (13) para,para-diamino-diphenyl methane, (14) phenylhydrazine, (15) amylamine, (16) aniline, (17) diaminamine, and (18) hexamethylenetetramine. Other amines somewhat less effective under the same conditions for the purpose than the foregoing are the following:

Table I

|   | Amine                         | Stained after— | Days |     |
|---|-------------------------------|----------------|------|-----|
|   |                               |                | Pho. | Am. |
| 1 | Tetramethyl thiuram disulfide | 89             |      |     |
| 2 | Para-phenetidine              | 81             |      |     |
| 3 | Ethyl alphanaphthylamine      | 54             |      |     |
| 4 | Ortho-aminodiphenyl           | 54             |      |     |
| 5 | Ortho-aminophenol             | 54             |      |     |
| 6 | Methyl anthranilic acid       | 29             |      |     |
| 7 | Dibeta naphthylamine          | 26             |      |     |
| 8 | Para-ultraniline              | 26             |      |     |

The mineral oil compositions used in the foregoing tests contained, as stated above, 0.25 per cent of the organic phosphite and 0.05 per cent or less (depending upon solubility) of the organic amine. These mineral oil compositions may be formed by adding the phosphite and the amine to the oil independently, but it is preferable to have the phosphite and the amine previously blended as a mineral oil-improving agent, thus safeguarding against deterioration of the phosphite prior to its incorporation in the oil. Composite mineral oil-improving agents to form oil blends of the foregoing types would consist of about 100 parts by weight of the phosphite and 20 parts or less of the amine, the improving agent being added to the oil in amounts of about .30 per cent or less, depending upon the amine content.

## EXAMPLE 2

As mentioned above, cyclohexylamine, orthotoluidine, and triethanolamine were among the most effective stabilizers observed. In order to differentiate between these compounds the storage temperature was raised to 160° F. and the following results were then obtained in a twenty-one day test period, using as a base oil an S. A. E. 20 oil. The phosphite used in this test was tri-para-tertiary amyl phenyl phosphite. In Table II below the three amines tested are indicated as follows: "Cyc." (cyclohexylamine), "Ort." (orthotoluidine), and "Triet." (triethanolamine). Under the heading "Per cent concentration in oil" are indicated the concentration of the phosphite (Pho.), the concentration of the amine (Am.) and the concentration of the improving agent (I. A.) (phosphite and amine composition) all as per cent by weight in the oil. Under the heading "Proportions in improving agent" are given the proportions in parts by weight of the phosphite (Pho.) and amine (Am.) which go to make up the particular improving agent under test.

Table II

| Amine  | Percent concentration in oil |       |       | Proportions in improving agent |     | Storage at 160° F., results | 5  |
|--------|------------------------------|-------|-------|--------------------------------|-----|-----------------------------|----|
|        | Pho.                         | Am.   | I. A. | Pho.                           | Am. |                             |    |
| Cyc.   | 0.25                         | 0.01  | 0.26  | 100                            | 4.0 | No stain (21 days).         |    |
| Cyc.   | 0.25                         | 0.005 | 0.255 | 100                            | 2.0 | No stain (21 days).         | 10 |
| Cyc.   | 0.25                         | 0.001 | 0.251 | 100                            | 0.4 | Stain (21 days).            |    |
| Ort.   | 0.25                         | 0.01  | 0.26  | 100                            | 4.0 | Stain (3 days).             |    |
| Ort.   | 0.25                         | 0.005 | 0.255 | 100                            | 2.0 | Stain (3 days).             |    |
| Ort.   | 0.25                         | 0.001 | 0.251 | 100                            | 0.4 | Stain (3 days).             |    |
| Triet. | 0.25                         | 0.01  | 0.26  | 100                            | 4.0 | Stain (6 days).             |    |
| Triet. | 0.25                         | 0.005 | 0.255 | 100                            | 2.0 | Stain (6 days).             |    |
| Triet. | 0.25                         | 0.001 | 0.251 | 100                            | 0.4 | Stain (3 days).             |    |
| None   | 0.25                         | —     | —     | 100                            | 0.0 | Stain (3 days).             | 15 |

## EXAMPLE 3

It has been mentioned above that the deterioration of an ester of phosphorous acid in a motor oil, for instance, is accompanied by a darkening of the oil as well as by staining if the oil is stored in a metal container, particularly a tin-coated container, where it is easily visible by contrast. The effectiveness of cyclohexylamine for stabilizing an ester of phosphorous acid in an oil against such deterioration and its accompanying effect upon darkening of the oil is shown by the data in Table III below in which the "phosphite" was tripara-tertiary amyl phenyl phosphite and in which the "amine" was cyclohexylamine.

Table III

| Oil blend                                        | Color after 21 days' storage at 160° F. in tinned container | 35       |  |
|--------------------------------------------------|-------------------------------------------------------------|----------|--|
|                                                  |                                                             | Lovibond |  |
| S. A. E. 20 oil+0.25% phosphite                  | 125                                                         | 125      |  |
| S. A. E. 20 oil+0.25% phosphite and 0.01% amine  | 100                                                         | 40       |  |
| S. A. E. 20 oil+0.25% phosphite and 0.005% amine | 105                                                         |          |  |

## EXAMPLE 4

In the foregoing examples it will be observed that the phosphites used were aryl phosphites. As has been previously pointed out, all known esters of phosphorous acid or organic phosphites are inherently unstable and our invention contemplates any suitable compound from this whole class as one constituent of the oil-improving agent or the improved mineral oil composition. Other representative phosphites which may be used are the alkyl phosphites, particularly the trialkyl phosphites, of which tributyl phosphite and tri-allyl phosphite are representative examples. The stain inhibiting action of amines on alkyl phosphites is demonstrated by Table IV below, which shows the results of a 150-160° F. storage test on S. A. E. 20 motor oil, using dicyclohexylamine ("Dicyc.") as the amine and tri-isoamyl phosphite as the phosphite ("Alk. Pho."). The various headings in the table have the same significance as in Table II.

Table IV

| Amine  | Percent concentration in oil |       |       | Proportions in improving agent |     | Storage at 160° F., results | 65 |
|--------|------------------------------|-------|-------|--------------------------------|-----|-----------------------------|----|
|        | Alk. pho.                    | Am.   | I. A. | Alk. pho.                      | Am. |                             |    |
| None   | 0.25                         | —     | 0.25  | 100                            | 0.0 | Stain (3 days).             | 70 |
| Dicyc. | 0.25                         | 0.015 | 0.265 | 100                            | 6.0 | No stain (6 days).          |    |

## EXAMPLE 5

The term "organic phosphite" used herein, as we have previously stated, is intended to be inclusive of thiophosphites. The stain-inhibiting 5 action of amines upon the thiophosphites is demonstrated by Table V below, which shows the results of a storage test at 150°-160° F. on S. A. E. 20 motor oil, using dicyclohexylamine ("Dicyc.") as the amine and triphenyl trithiophosphite 10 ("Thiophos.") as the phosphite. The various headings in the table have the same significance as in Table II.

Table V

| Amine      | Percent concentration in oil |       |       | Proportions in improving agent |     | Storage at 160° F., results |
|------------|------------------------------|-------|-------|--------------------------------|-----|-----------------------------|
|            | Thio-phos.                   | Am.   | I. A. | Thio-phos.                     | Am. |                             |
| None.....  | 0.25                         |       | 0.25  | 100                            | 0.0 | Stain (1 day).              |
| Dicyc..... | 0.25                         | 0.015 | 0.265 | 100                            | 6.0 | No stain (4 days).          |

25 It is to be understood that while we have herein given certain specific examples of phosphites and amines, such examples are for illustration only. The invention is not limited to any particular phosphite or amine or to any particular 30 combinations of phosphites and amines but includes within its scope such variations and modifications as fairly come within the spirit of the appended claims.

We claim:

35 1. A lubricating oil composition comprising a major proportion of a mineral lubricating oil, a minor proportion of an ester of phosphorous acid, which would normally tend to stain tin-coated metal containers, and a small amount, sufficient 40 to bring about substantial stability of said ester and retard such staining action, of an oil-soluble organic amine.

45 2. A lubricating oil composition comprising a major proportion of a mineral lubricating oil, a minor proportion of an ester of phosphorous acid, which would normally tend to stain tin-coated metal containers, and a small amount, sufficient 50 to bring about substantial stability of said ester and retard such staining action, of a material selected from the group consisting of cyclohexylamine; dicyclohexylamine; lecithin; morpholine; orthotolidine; triethanolamine, triethanolamine stearate; para-phenylene diamine; para-toluidine; beta naphthylamine; dianisidine; orthotolidine; para,para-diamino diphenyl methane; phenyl hydrazine; amyl amine; aniline; diamylamine; hexamethylenetetramine.

55 3. A lubricating oil composition comprising a major proportion of a mineral lubricating oil, a minor proportion of an ester of phosphorous acid, which would normally tend to stain tin-coated metal containers, and a small amount, sufficient 60 to bring about substantial stability of said ester and retard such staining action, of a cyclohexylamine.

65 4. A lubricating oil composition stable against deterioration when stored in tin-coated containers comprising a major proportion of mineral lubricating oil, a minor proportion of an ester of phosphorous acid, which normally tends to stain such containers, and not more than about 0.05 per cent by weight of an oil-soluble organic amine.

70 5. A lubricating oil composition, stable against deterioration when stored in tin-coated con-

75 tainers, comprising a major proportion of mineral lubricating oil, a minor proportion of an aryl phosphite, and not more than 0.05 per cent by weight of an oil-soluble organic amine.

80 6. A lubricating oil composition stable against 85 deterioration when stored in tin-coated containers comprising a major proportion of mineral lubricating oil, a minor proportion of an alkyl phosphite, and not more than 0.05 per cent by weight of an oil-soluble organic amine. 10

85 7. A lubricating oil composition stable against 15 deterioration when stored in tin-coated containers comprising a major proportion of a mineral lubricating oil, a minor proportion of an organic phosphite, and not more than 0.05 per cent by weight of a cyclohexylamine. 15

90 8. A lubricating oil composition comprising a major proportion of a mineral lubricating oil, a minor proportion of a triaryl phosphite, and from 0.001 to 0.01 per cent of a cyclohexylamine. 20

95 9. A lubricating oil composition comprising a major proportion of a mineral lubricating oil, a minor proportion of a triester of phosphorous acid and a small amount, sufficient to bring about substantial stability of the said triester, of an oil-soluble organic amine. 25

100 10. A lubricating oil composition comprising a major proportion of a mineral lubricating oil, a minor proportion of a triester of phosphorous acid and a small amount, sufficient to bring about 30 substantial stability of the said triester, of an oil-soluble organic amine selected from the group consisting of cyclohexylamine; dicyclohexylamine; lecithin; morpholine; orthotolidine; triethanolamine; triethanolamine stearate; para-phenylene diamine; para-toluidine; beta naphthylamine; dianisidine; orthotolidine; para,para-diamino diphenyl methane; phenyl hydrazine; amyl amine; aniline; diamylamine; hexamethylenetetramine. 35

105 11. A lubricating oil composition comprising: a major proportion of a mineral lubricating oil; a minor proportion of an organic phosphite selected from the group consisting of triamyl-phenyl phosphite, tributyl phenyl phosphite, 45 triphenyl phosphite, tricresyl phosphite, tributyl phosphite, and triamyl phosphite, and a small amount, sufficient to bring about substantial stability of the phosphorus compound, of an oil-soluble organic amine. 40

110 12. A lubricating oil composition comprising: a major proportion of a mineral lubricating oil; a minor proportion of an organic phosphite selected from the group consisting of triamyl-phenyl phosphite, tributyl phenyl phosphite, triphenyl phosphite, tricresyl phosphite, tributyl phosphite, triamyl phosphite; and a small amount, sufficient 50 to bring about substantial stability of the phosphorus compound, of an oil-soluble organic amine selected from the group consisting of cyclohexylamine, dicyclohexylamine, lecithin, morpholine, orthotolidine, triethanolamine, triethanolamine stearate, para-phenylene diamine, para-toluidine, beta naphthylamine, dianisidine, orthotolidine, para,para-diamino diphenylmethane, phenyl hydrazine, amyl amine, aniline, diamylamine, hexamethylenetetramine. 55

115 13. A lubricating oil composition comprising: a major proportion of a mineral lubricating oil; a minor proportion of a phosphorus compound selected from the group consisting of triamyl-phenyl phosphite, tributyl phenyl phosphite, tricresyl phosphite, triphenyl phosphite, tributyl phosphite, and triamyl phosphite; and a small amount, sufficient 60 to bring about substantial stability of the phosphorus compound, of an oil-soluble organic amine selected from the group consisting of cyclohexylamine, dicyclohexylamine, lecithin, morpholine, orthotolidine, triethanolamine, triethanolamine stearate, para-phenylene diamine, para-toluidine, beta naphthylamine, dianisidine, orthotolidine, para,para-diamino diphenylmethane, phenyl hydrazine, amyl amine, aniline, diamylamine, hexamethylenetetramine. 65

120 14. A lubricating oil composition comprising: a major proportion of a mineral lubricating oil; a minor proportion of a phosphorus compound selected from the group consisting of triamyl-phenyl phosphite, tributyl phenyl phosphite, tricresyl phosphite, triphenyl phosphite, tributyl phosphite, and triamyl phosphite; and a small amount, sufficient 70 to bring about substantial stability of the phosphorus compound, of an oil-soluble organic amine selected from the group consisting of cyclohexylamine, dicyclohexylamine, lecithin, morpholine, orthotolidine, triethanolamine, triethanolamine stearate, para-phenylene diamine, para-toluidine, beta naphthylamine, dianisidine, orthotolidine, para,para-diamino diphenylmethane, phenyl hydrazine, amyl amine, aniline, diamylamine, hexamethylenetetramine. 75

bility of the phosphorus compound, of a cyclohexylamine.

5 14. An improving agent for mineral oils and the like comprising an ester of phosphorous acid and in admixture therewith an oil-soluble organic amine in an amount from about 0.25 per cent to about 50 per cent of the weight of said ester.

10 15. An improving agent for mineral oils and the like comprising an ester of phosphorous acid and in admixture therewith an oil-soluble organic amine in an amount from about 0.4 per cent to about 20 per cent the weight of said ester.

15 16. An improving agent for mineral oils and the like comprising an ester of phosphorous acid and in admixture therewith an oil-soluble organic amine in an amount from about 0.4 per cent to about 4.0 per cent the weight of said ester.

20 17. An improving agent for mineral oils and the like comprising an ester of phosphorous acid and in admixture therewith from about two to about three per cent by weight of a cyclohexylamine.

18. An improving agent for mineral oils and the

like comprising a triester of phosphorous acid and in admixture therewith from about 0.4 per cent to about 20 per cent by weight of an oil-soluble organic amine.

19. An improving agent for mineral oils and the like comprising an organic phosphite selected from the group consisting of: triphenyl phosphite, tricresyl phosphite, triamyl phenyl phosphite, tributyl phenyl phosphite, triamyl phosphite, and tributyl phosphite and in admixture therewith from about 0.4 per cent to about 20 per cent of an oil-soluble organic amine.

20 20. An improving agent for mineral oils and the like comprising an organic phosphite selected from the group consisting of: triphenyl phosphite, tricresyl phosphite, triamyl phenyl phosphite, tributyl phenyl phosphite, triamyl phosphite, and tributyl phosphite and in admixture therewith from about two per cent to about three per cent by weight of a cyclohexylamine.

ROBERT C. MORAN.

ALFRED P. KOZACIK.